

## UNITED STATES PATENT OFFICE.

GILLES HOLST, EKKO OOSTERHUIS, AND JOHANNES BRUIJNES, OF EINDHOVEN, NETHERLANDS, ASSIGNORS TO NAAMLOOZE VENNOOTSCHAP PHILIPS' GLOEILAMPEN-FABRIEKEN, OF EINDHOVEN, NETHERLANDS.

## ELECTRIC DISCHARGE TUBE.

No Drawing.

Application filed June 1, 1922. Serial No. 565,230.

*To all whom it may concern:*

Be it known that we, GILLES HOLST, EKKO OOSTERHUIS, and JOHANNES BRUIJNES, all subjects of the Queen of the Netherlands, 5 residing at Eindhoven, in the Province of North Brabant, in the Kingdom of the Netherlands, have invented certain new and useful Improvements in or Relating to Electric Discharge Tubes, of which the following is a specification.

This invention relates to electric discharge tubes in which a discharge is effected in a suitable gas-filling between electrodes which—at least at starting the tube—have 15 a relatively low temperature such that they do not independently emit electrons.

In gas-filled electric discharge tubes of this kind it has always been difficult to start the discharge without auxiliary devices, 20 which enable the tube to be worked on the tension available on ordinary electric mains.

It is known to facilitate the starting of the discharge, by making the cathode of suitable material and by giving it a suitable 25 construction. It has also been proposed to add a small proportion of non-rare gases or vapours to the gas-filling, but this has been chiefly for the purpose of counteracting the disintegration of the cathode and prolonging the life of the lamp. This latter result 30 is obtained with various mixtures of gases without however lowering the starting potential. According to the present invention rare gases are added to a principal filling of rare gas for the purpose of reducing the 35 starting potential of discharge tubes having independent discharge. An independent discharge is an electric discharge which is started simply by supplying a suitable alternating or direct current-tension to the electrodes without requiring cathode incandescence or any auxiliary device to liberate electrons or ions in the path of the discharge 40 such as characterize X-rays or ultraviolet rays.

The conditions to be imposed on the composition of the gas-filling necessary to ensure the ignition of the tube on the tension

of ordinary electric mains have now been recognized and the invention relates to an 50 electric discharge tube in which the starting potential is lowered by a special composition of the gas-filling. To that end the gas-filling of the tube consists principally of one gas and an added small quantity of 55 another gas having an ionization potential lower than the tension at which the first inelastic collision in the first mentioned gas occurs.

It has been found that when the gas-filling 60 of the tube is composed as above described, discharge tubes of any type may be started at ordinary electric main tensions independently of the shape or nature of the electrodes.

It is quite likely that if the tube were filled 65 exclusively with the gas used in this invention as an addition, all electrons in the said gas would lose their energy in inelastic collisions before the ionization potential were 70 reached, so that no discharge would take place. If however this gas is in but a small proportion in another gas the resonance potential of which is much higher, a large portion 75 of the electrons has no opportunity of coming into resonance so that it can effect a discharge when the ionization potential is reached. For example, no discharge is produced either in neon or in argon at a tension of 220 volts in a tube in which the electrodes are about 5 cm. apart and the gas pressure is 1 cm. If however the tube is filled with neon to which 0.5 to 5% of argon is added, a discharge is produced at the same tension. The same result is obtained (even 80 if the proportions of the mixture are altered) in mixtures of gases in which a small quantity of neon, argon or crypton is added to the principal volume of helium, or in which an addition of crypton is made to argon as the principal component.

The invention is applicable to gas-filled 85 electric discharge tubes of any type, that is to say gas lamps or glow discharge lamps as well as rectifiers, amplifiers and the like.

What we claim is:

1. A gas-filled electric discharge tube with independent discharge in which the gas-filling consists of a principal volume of one rare gas and an added small quantity of an-  
5 other rare gas the ionization potential of which is lower than the potential at which the first inelastic collision in the first men-  
tioned gas occurs.
2. An electric discharge tube, filled with neon to which 0.5 to 5% argon is added. 10  
In testimony whereof we have affixed our signatures.

GILLES HOLST.  
EKKO OOSTERHUIS.  
JOHANNES BRUIJNES.